

## UNITED STATES PATENT OFFICE

2,355,009

## LUBRICANT

Arnold J. Morway, Clark Township, Union County, and John C. Zimmer, Union, N. J., assignors to Standard Oil Development Company, a corporation of Delaware

No Drawing. Application October 4, 1941,  
Serial No. 413,650

8 Claims. (Cl. 252—40)

The present invention is concerned with the production of improved lubricating grease compositions. The invention more particularly relates to a grease composition which is especially adapted for use under extreme variations in climatic conditions, such as wide variations in temperature and humidity. The preferred composition comprises a mineral oil base thickened to a grease consistency with a mixture of saturated fatty acid soaps of lithium and barium.

It is known in the art to prepare various lubricating grease compositions adapted for particular uses. The uses in which grease compositions are employed present a wide variety of conditions and generally a grease prepared with a given set of conditions in mind is not suitable for use under a different set of conditions. Airplanes are controlled in flight by special mechanisms such as rudder, elevators, and ailerons which are adapted to the main portions of the airplane such as fuselage and wings by specially designed hinges. These hinges have metal to metal contact bearing surfaces which offer a very difficult lubrication problem. Airplanes are operated under the most severe changes in climatic conditions and since the failure of even one part of the mechanism might well result in a catastrophe, it is imperative that all parts of the plane be maintained in as perfect a mechanical condition as possible. In order to be in good mechanical condition all movable parts should be free and well lubricated at all times. It is not uncommon for a plane during a single trip to be subjected to extremely high ground temperatures, subzero temperatures in the upper atmosphere as well as conditions of high humidity such as rain, snow, or ice. Any lubricant used upon the control mechanisms of the plane must be capable of withstanding these conditions without disintegration.

High temperature greases such as the sodium soap greases are known to the art, however they are quite water-soluble and readily disintegrate under humid conditions. Water-insoluble greases, such as the calcium soap greases, are also known, but these compositions will not withstand high temperatures. Aluminum soap greases are also water-insoluble but have a relatively low transient point where they become fluid and run out of the bearing. Barium soap greases are only slowly affected by the presence of water and effectively withstand elevated temperatures but have the disadvantages of losing their grease structure on standing at lower temperatures and becoming quite stiff and heavy at elevated temperatures.

It is an object of this invention to produce a grease composition which will provide adequate lubrication at both high and low temperatures and will not decompose in the presence of excess-

sive moisture. This and other objects will be apparent to those skilled in the art upon reading the following description.

The grease composition made in accordance with the present invention comprises essentially a low pour point lubricating mineral oil distillate, a lithium soap of a saturated fatty acid and a barium soap of a saturated fatty acid, although it is preferred to use from 10 to 25% of the lithium soap and from 0.50 to 8% of the barium soap based upon the total composition. A small amount of an anti-oxidant, say 0.2%, such as phenyl alpha naphthylamine or a mixture of zinc naphthenate and phenyl alpha naphthylamine, may be used if desired.

Although any of the numerous types of low pour point lubricating oils may be used as the base for compositions made in accordance with this invention, it is preferred to use a Coastal type oil having a viscosity, in the range of from about 58 seconds to 100 seconds S. U. V. at 100° F. and a cold test below 40° F.

For the formation of the soaps utilized in the production of the greases any saturated fats or saturated fatty acids derived therefrom, such as stearin or stearic acid may be used, although it is preferred to use the saturated acids derived from hydrogenated fish oil.

Any of the methods customarily employed in the compounding of greases may be used in the production of the compositions of this invention. The soaps may be produced separately and then mixed with the oil by heat and agitation; or preferably the saturated fat or fatty acid to be combined with the lithium and barium may be dissolved in a portion of the lubricating oil by heating the oil sufficiently to dissolve the fat or acid in the oil, reacting the fat or fatty acid with lithium and barium hydroxides and then the remainder of the lubricating oil is added after which the mixture is brought to a clear solution by heating, and stirring, generally to a temperature between 360° and 400° F., the anti-oxidant added and the mixture stirred until cool. Greases of varying consistency to meet the demands of particular conditions may be secured by varying the soap content of the grease within the limits specified. The following examples will serve to illustrate specific embodiments of the invention.

## Example 1

|                                                     | Per cent |
|-----------------------------------------------------|----------|
| Hydrogenated fish oil acids                         | 19.00    |
| Barium hydroxide ( $Ba(OH)_2 \cdot 8H_2O$ )         | 1.00     |
| Lithium hydroxide (54% LiOH)                        | 2.50     |
| Lubricating oil (low pour Coastal oil)              | 38.75    |
| Lubricating oil (low viscosity, low pour point oil) | 38.75    |
| Phenyl alpha naphthylamine                          | 0.2      |

In compounding the above formula the acid and approximately  $\frac{1}{4}$  of the oil are charged into a fire-heated kettle equipped with agitators. The mixture is then heated and stirred to a temperature of about 150° F. or until all the acid is melted and dissolved in the oil and then the lithium hydroxide, dissolved in boiling water, is added to the acid-oil solution. Heating and agitation is continued and the temperature permitted to slowly rise until it reaches about 200° F. The barium hydroxide, dissolved in boiling water is then added and the heating and stirring continued along with intermittent additions of lubricating oil until all of the oil has been included and the temperature reaches about 360° F. At this point the grease is of a fibrous rubbery structure. Heating is continued until the grease becomes fluid, about 380° F. The anti-oxidant is then added, heating discontinued and the stirring continued until the grease has cooled to below 180° F. The grease is of an excellent smooth structure having the following characteristics.

Free acidity (A. S. T. M.) per cent (as oleic acid) \_\_\_\_\_ 0.68  
 A. S. T. M. dropping point \_\_\_\_\_ °F 380  
 A. S. T. M. penetration at 77° F. \_\_\_\_\_ 240  
 A. S. T. M. worked penetration at 77° F. \_\_\_\_\_ 265

About 1% of water can be worked into the grease, by beating in the presence of a relatively large amount of water, however this water will run off when the grease is allowed to stand for a few hours and again worked.

*Example 2*

|                                                                                | Per cent |
|--------------------------------------------------------------------------------|----------|
| Stearic acid                                                                   | 15.00    |
| Barium hydroxide Ba(OH) <sub>2</sub> · 8H <sub>2</sub> O                       | 0.79     |
| Lithium hydroxide                                                              | 1.97     |
| Zinc naphthenate                                                               | 0.40     |
| Phenyl alpha naphthylamine                                                     | 0.40     |
| Acid treated low cold test transformer oil (58° S. S. U. viscosity at 100° F.) | 81.44    |

The same method of manufacture is used as that described in Example 1. However the inhibitor (phenyl alpha naphthylamine) and zinc naphthenate are added last at approximately

360° F. The kettle must be equipped with a condenser to prevent the boiling off of the light hydrocarbon oil used.

5 Free acidity \_\_\_\_\_ per cent (as oleic acid) 0.43  
 A. S. T. M. dropping point \_\_\_\_\_ °F 360  
 Penetration \_\_\_\_\_ 300  
 Worked penetration \_\_\_\_\_ 320

What is claimed is:

1. An improved lubricating grease composition comprising a low pour point lubricating mineral oil distillate, a mixture of lithium and barium soaps of saturated fatty acids in which the amount of lithium soap exceeds the amount of barium soap.

2. A composition as defined in claim 1 in which the lithium soap is the lithium soap of hydrogenated fish oil acids.

3. A composition as defined by claim 1 in which the saturated fatty acids are the acids derived from hydrogenated fish oil.

4. An improved lubricating grease composition comprising a low pour point, low viscosity, lubricating mineral oil distillate and a mixture of lithium and barium soaps of saturated fatty acids in which the amount of lithium soap exceeds the amount of barium soap.

5. An improved lubricating grease composition comprising from 67 to 89.5% of a low pour point, low viscosity lubricating mineral oil distillate, from 10 to 25% of a lithium soap of a saturated fatty acid and from 0.5 to 8% of a barium soap of a saturated fatty acid.

6. A composition as defined by claim 5 in which the lithium soap is the lithium soap of hydrogenated fish oil acids.

7. A composition as defined by claim 5 in which the fatty acids are the acids obtained from hydrogenated fish oil.

8. An improved lubricating grease composition consisting of 77.5% of a low viscosity, low pour mineral lubricating oil, 18% of lithium soaps of hydrogenated fish oil acids, 7.5% barium soaps of hydrogenated fish oil acids and 0.2% phenyl alpha naphthylamine.

ARNOLD J. MORWAY.  
 JOHN C. ZIMMER.